

## UNITED STATES PATENT OFFICE.

NATHANIEL A. THOMPSON, OF KANSAS CITY, KANSAS.

## WATERPROOFING FOR CLOTH.

No Drawing. Original application filed March 8, 1923, Serial No. 623,725. Divided and this application filed March 8, 1923. Serial No. 623,727.

To all whom it may concern:

Be it known that I, NATHANIEL A. THOMPSON, a citizen of the United States, residing at Kansas City, in the county of Wyandotte and State of Kansas, have invented certain new and useful Improvements in Waterproofing for Cloth, of which the following is a specification.

The object of this invention is to make a more perfect water-proofing for cloth that will turn the water under any conditions of weather. Cloth treated by this process has its period of life increased for not only is the fabric protected from moisture but the ingredients that render it water-proof have no deleterious effect on the fibre.

Because of the excellent water-proofing action of the ingredients as used in my process, the cloth is not as stiff as is the case with ordinary water-proofing goods, for a thinner coating accomplishes the same result.

Another object of my process is to produce a cloth which will be absolutely impervious to water and will not crack when folded.

With these and other objects in view, the invention consists of a process as herein set forth, with the understanding that the several necessary elements entering into the composition may be varied in proportion without departing from the nature and scope of the invention.

To make the water-proofing, a small quantity of rubber is cooked in boiling oil until the rubber has become thoroughly dissolved. Any of the heavier hydrocarbon oils may be used or a vegetable oil, as linseed or cotton seed oil. The vegetable oils have been found to be superior to the mineral oils, but it will be understood that the invention is not limited to the exact type of oil used.

To the hot mixture of oil and rubber is added a small quantity of asphalt. To this mixture is then added a finely comminuted filler, such as pulverized calcium carbonate or ferric oxide. The exact composition of the body does not form part of this invention as any of the insoluble mineral salts or oxides accomplish the same result.

It has been found by actual experiment

that good proportions of the ingredients used are as follows:

|         | Per cent. |    |
|---------|-----------|----|
| Oil     | 40 to 50  | 55 |
| Rubber  | 5 to 10   |    |
| Asphalt | 5 to 10   |    |
| Filler  | 30 to 50  |    |

The stiffness of the compound is determined by the proportion of filler added.

The rubber has the property of acting as a binder to keep the asphalt from separating from the oil which would otherwise be its tendency when allowed to stand. The asphalt likewise keeps the finely ground filler in solution and does not allow it to precipitate. Thus it will be seen that the greater the amount of ground filler added the greater the amount of asphalt necessary and likewise the greater the quantity of rubber. The rubber has the complementary effect on the asphalt that the asphalt has on the filler, i. e., that of holding it in solution or of forming a blend. When the water-proofing composition has been prepared a proper coloring may be given to it by means of any suitable pigment.

The water-proofing composition may be applied to the fabric by means of a brush or roller and the fabric is allowed to dry or set from nine to eleven days. The composition has a tendency to become very viscous, due, it is thought, to the oxidizing influence of the air and at the end of nine or eleven days, depending on the temperature and proportion of ingredients used in the composition, the fabric is coated with a water-proofing that is absolutely and uniformly impervious to water because of the perfect blend between the different constituents and the even grade of the compound, regardless of the length of time it has remained in the container.

Having set forth my invention, what I claim is:—

1. A water-proofing composition composed of a heavy hydro-carbon oil, asphalt, rubber and a filler.

2. A water-proofing composition composed of a heavy hydro-carbon oil, approximately 40 to 50 per cent, rubber 5 to 10 per

cent, asphalt 5 to 10 per cent, and a filler 30 to 50 per cent.

3. A process for making water-proofing composition consisting of boiling a heavy hydro-carbon oil with rubber, adding asphalt and then adding a filler.

4. A process for making a water-proofing

composition consisting of boiling 40 to 50 parts of heavy hydro-carbon oil with 5 to 10 parts rubber, adding 5 to 10 parts asphalt and then adding a filler of thirty to fifty parts.

In testimony whereof I affix my signature.

NATHANIEL A. THOMPSON.